

(No Model.)

J. B. & C. Z. DE YOUNG.

MAT.

No. 249,317.

Patented Nov. 8, 1881.

Fig. 1.



Fig. 2.



WITNESSES:

*A. S. Grant*  
*A. F. Kicher*

INVENTORS:

*Joseph B. De Young*  
*W. J. De Young*  
*John C. Diederich*  
BY *John C. Diederich* ATTORNEY.

# UNITED STATES PATENT OFFICE.

JOSEPH B. DE YOUNG AND CHARLES Z. DE YOUNG, OF PHILADELPHIA, PA.

## MAT.

SPECIFICATION forming part of Letters Patent No. 249,317, dated November 8, 1881.

Application filed June 16, 1881. (No model.)

*To all whom it may concern:*

Be it known that we, JOSEPH B. DE YOUNG and CHARLES Z. DE YOUNG, both citizens of the United States, residing in the city and county of Philadelphia, and State of Pennsylvania, have invented a new and useful Improvement in Mats, which improvement is fully set forth in the following specification and accompanying drawings, in which—

10 Figure 1 is a face view of the mat embodying our invention. Fig. 2 is a side edge view thereof.

Similar letters of reference indicate corresponding parts in the two figures.

15 Our invention consists of a woven mat formed partly or entirely of disintegrated corn-husk, which will be found to be strong, durable, and serviceable.

Referring to the drawings, A represents the mat, which is formed entirely or partly of disintegrated corn-husk.

We may weave the mat in any suitable manner, employing corn-husk fiber as warp, filling, and topping, or we may use jute or other fiber 25 for either the warp or filling, or for both the warp and filling, with the corn-husk fiber for the topping or surface of the mat. We may weave the mat on the tufted principle or on the rod principle, and other modes of weaving may 30 be adopted, as the husk may be readily worked, the product in any case having its top or wiping surface of corn-husks.

Corn-husk in a green state consists of fiber and integument, which latter is tough and pliable, but in a dry state is harsh and brittle. Disintegrated corn-husk has the integument removed, leaving the fiber or staple long, pli-

able, and tough. When the fiber is woven into mats it produces a wiping or wearing surface which readily sustains itself, as the fiber is 40 pliable or elastic. After the mat has been used the fiber rights itself, whereby the surface of the mat is kept compact and a broken-down appearance of the mat is prevented. Furthermore, the disintegrated material or fiber is 45 tough and strong, whereby the mat is durable and renders good service, and its glossy, bright, and light appearance is imparted to the mat as an admirable quality thereof.

The clipping or finishing of the mat is read- 50ily accomplished, and as the material readily takes dye and may be bleached, it is evident that the mats may be produced in various colors, always presenting bright appearances.

By the use of the present material we utilize 55 a product of this country, unlike cocoa fiber, which is imported, and create a new industry, which enhances the value of corn-husk.

We are aware that mats have been made from corn-husks, and disclaim the same, broad- 60ly; but we are not aware of any mat made of disintegrated corn-husk wherein the harsh and brittle integument is removed and the valuable fiber is preserved; wherefore

We claim as new—  
As a new article of manufacture, a woven mat having its top or wiping surface formed of disintegrated corn-husk, substantially as 65 and for the purpose set forth.

JOSEPH B. DE YOUNG.  
CHAS. Z. DE YOUNG.

Witnesses:

JOHN A. WIEDERSHEIM,  
W. F. KIRCHER.